

## UNITED STATES PATENT OFFICE

LUDWIG KERN AND FERNANDO C. KERN, OF WEBSTER GROVES, MISSOURI

## PROCESS OF COKING SOLID CARBONIZABLE MATERIAL

No Drawing.

Application filed June 18, 1930. Serial No. 462,126.

This invention relates to coke, and with regard to certain more specific features, to smokeless coke and the manufacture thereof.

Among the several objects of the invention 5 may be noted the provision of a process for the manufacture of smokeless coke of a hard-wear-resisting, homogeneous character; a process wherein smoke producing binder materials are eliminated; a process wherein the 10 natural gangue constituents of a coal are utilized as a basis for the binder material for said coal; a process which includes an economical low-temperature distillation; and a process of the class described which is easily 15 and economically carried through and which yields products of great commercial value. Other objects will be in part obvious and in part pointed out hereinafter.

The invention accordingly comprises the 20 elements and combinations of elements, steps and sequence of steps and features of synthesis which will be exemplified in the description hereinafter and the scope of the application of which will be indicated in the 25 following claims.

It has been found that coal, when ground to a sufficient fineness, is mechanically separated or detached into gangue constituents and carbonaceous constituents. The gangue constituents herein referred to are those occluded in the coal, and not those chemically combined. Occluded gangue constituents form a preponderant majority of the total gangue 30 constituents, those chemically combined being present only in relatively small quantities. This phenomena, in general, takes places at a fineness of 150 mesh or finer. In finely comminuted coal, therefore, there is present in intimate mixture comminuted gangue constituents and comminuted carbonaceous materials.

We have found that the comminuted gangue constituents, when treated with alkaline solutions, form a plastic binding material 45 or cement which, with suitable homogenizing, serves to plasticize or bind the carbonaceous particles into a firm, moldable mass. The plasticized gangue constituents apparently form a shell or jacket for each carbon particle. 50 The plastic carbonaceous mass is preferably

molded into shapes or briquettes (if the shape of the product is not necessarily regular, specific molding is not necessary), dried, and the dried briquettes subjected to either a high-temperature or a low-temperature distillation or carbonization. In the course of the carbonization, the shells around the carbonaceous particles harden to strengthen the product generally, but remain sufficiently porous to permit the evolution of volatile 55 products. The hardened shells of gangue constituents further serve to bind the carbonaceous particles, thereby preventing inordinate swelling and bulging, and consequent irregularity of product shape. These 60 shells also prevent adjacent particles of carbonaceous material from adhering to each other during the plastic state of said particles (at about 400° C.), and from adhering to the 65 walls of the retort. The gangue constituents 70 are not present in objectionable quantities in the coke product, and, furthermore, in the burning of the product coke, these gangue constituents are reduced to a readily-pulverized ash which does not clinker and prove 75 otherwise objectionable.

Alkaline solutions are particularly valuable as plasticizing agents when the gangue constituents are predominantly siliceous in character. Examples of the alkaline solutions which may be satisfactorily used include sodium hydroxide, sodium carbonate, ammonium hydroxide, and the like.

As an example of our process, the following is cited:

Bituminous Illinois coal is ground to a fineness of 150 mesh or finer, and to the powdered coal is added from 10 to 30 per cent, by weight, of a water solution of sodium hydroxide of gravity 1° to 5° Bé. The mixture is then ground in a pug mill, wet pan, or other convenient mixing or kneading device until it is formed into a homogeneous plastic mass of pasty consistency. The plastic mass is then shaped into briquettes, for example, in an auger extrusion machine. The briquettes are preferably allowed to dry, and then charged into a carbonization retort. The temperature is gradually brought to a 90 temperature of the order of 600° C., with 95 100

attendant evolution of hydrocarbons and the like, which are preferably collected and condensed according to methods known to the art. After carbonization is complete, the 5 briquettes are removed and cooled or quenched.

The product is a homogeneous, even-burning, smokeless, hard coke briquette, which is adapted for use as a commercial or home fuel.

10 In view of the foregoing, it will be seen that the several objects of the invention are achieved and other advantageous results attained.

15 As many changes could be made in carrying out the above objects without departing from the scope of the invention, it is intended that all matter contained in the above description shall be interpreted as illustrative and not in a limiting sense.

20 We claim:

1. The process of coking solid carbonizable material having gangue constituents predominantly high in silica, comprising comminuting said material to an extent sufficient to 25 mechanically detach gangue constituents from said material, adding a plasticizing agent comprising an alkaline solution to said comminuted material, said alkaline solution reacting with the siliceous constituents 30 of said gangue material to form a binder for the remainder of said carbonizable material and thereby to plasticize the entire mass of comminuted material, subjecting the plastic mass to a destructive distillation, and thereby 35 forming coke.

2. The process of coking solid carbonizable material having gangue constituents predominantly high in silica, comprising comminuting said material to an extent sufficient to 40 mechanically detach gangue constituents from said material, adding a plasticizing agent comprising a solution of sodium hydroxide to said comminuted material, said sodium hydroxide reacting with 45 the siliceous constituents of said gangue material to form a binder for the remainder of said carbonizable material and thereby to plasticize the entire mass of comminuted material, subjecting the plastic mass to a destructive distillation, and thereby 50 forming coke.

In testimony whereof, we have signed our names to this specification this 13th day of June, 1930.

55

LUDWIG KERN.  
FERNANDO C. KERN.